

Jan. 6, 1942.

J. L. WOODBRIDGE

2,269,094

METHOD OF AND APPARATUS FOR MAKING LEAD OXIDE POWDER

Filed Sept. 29, 1938



WITNESS:

*Bob C. Mitchell*

INVENTOR

*Joseph Lester Woodbridge*

BY

*Augustus B. Strongton*  
ATTORNEY.

## UNITED STATES PATENT OFFICE

2,269,094

METHOD OF AND APPARATUS FOR MAKING  
LEAD OXIDE POWDER

Joseph Lester Woodbridge, Philadelphia, Pa., assignor to The Electric Storage Battery Company, Philadelphia, Pa., a corporation of New Jersey

Application September 29, 1938, Serial No. 232,352

9 Claims. (Cl. 23—146)

The objects of the present invention are to provide for the continuous manufacture of lead oxide powder at comparatively little cost and in increased quantity.

Another object of the invention is to provide an apparatus by means of which the process can be economically and satisfactorily practiced.

According to the present invention the surface of a strip or ribbon of lead is microscopically cracked and oxidized and scaled by disturbing or working the surface while the ribbon is at a high temperature and in the presence of air.

The invention comprises the improvements to be presently described and finally claimed.

In the following description reference will be made to the accompanying drawing forming part hereof and in which,

Figure 1 is a transverse sectional view of apparatus and also illustrative of the process of the present invention.

Figure 2 is a transverse sectional view taken on the line 2—2 of Figure 1.

Figure 3 is a sectional view taken on the line 3—3 of Figure 1.

Figure 4 is a side view illustrating a modification of the apparatus, and

Figure 5 is a similar view illustrating another modification.

The process will now be described in connection with the apparatus shown in Figure 1. Parts of the apparatus are repeated and a detailed description will be given of one of the parts and in the corresponding part the exponent *a* will be applied to the reference letters used. 1 is a receptacle or chamber of generally rectangular shape and it is shown as open at the top and bottom. 2 indicates a number of revoluble drums having corrugated surfaces. These drums are suitably driven and through them travels a strip or ribbon of lead 3. As shown the strip of lead or ribbon is produced by allowing a stream of molten lead from the melting pot 4 to pass out of the nozzle 5 onto a traveling belt 6 which passes around two drums 7 and 8. The drum 7 is provided with flanges 9 to confine the stream or ribbon of molten lead on either side until it has congealed. A spray of water 10 is directed onto the lead as it leaves the nozzle 5 to cause quick solidification. The strip or ribbon of lead 3 passes through the opening 11 into the receptacle 1 and thence downwardly between the various drums 2 at the left-hand side of the chamber 1 then across horizontally and upward around the various drums 2 on the right-hand side of the chamber 1 and out of the chamber 55

through the opening 12. From that point the strip of lead passes through the opening 11a of the second chamber 1a and finally the strip or ribbon passes out of the second chamber through the opening 12a from which point it passes into the melting pot 13. The lead in the melting pot 13 may be returned to the melting pot 4.

The strip of lead 3 is guided around the drums 2 by stationary guides 14. These guides are made of members spaced apart to permit fine powder which is detached from the lead ribbon to sift downward to the bottom of the chamber 1 where it is discharged through a hopper like opening into a suitable drum or receptacle 15. The stationary guide 14 is located beneath the horizontal portion of the lead strip or ribbon 3 and curves around the two bottom drums as shown. The guide 16 is of generally triangular form as shown in Figure 3 in order to shed powder settling down upon it so that the powder will fall into the drum 15. A supply of air which may be heated is furnished by means of a blower 25 equipped with a heater 18. The air is supplied through the vertical pipe 17 in which openings are provided opposite the stationary guides 14. Thus streams of heated air are directed upon the lead strip or ribbon.

As the lead strip passes through the apparatus its surface becomes oxidized and the fine oxidized particles are detached falling to the bottom of the chamber and into the receiving drum. The lead strip becomes attenuated but before it becomes so thin as to endanger its breaking into pieces of comparatively large size and while it is still in the form of a continuous ribbon it passes out of the final opening 12a in the last chamber and into the melting pot 13. In the modification shown in Figure 4 the lead ribbon 3b is conducted upon a conveyor 26 beneath rolls 19 which work its surface and past air injectors 20. As shown in Figure 5 the lead ribbon 3c is led past hammers or hammering devices 21 and over rolls 22. In the form of apparatus illustrated in Figures 4 and 5 the lead powder is delivered at the right-hand end. Referring to Figure 4, 23 indicates a device for controlling the flow of molten lead from the receptacle 24.

The principle involved is that when the surface of a piece of lead is deformed as by bending, crushing or otherwise the crystalline structure is broken up by the formation of inter-crystalline seams or crevices of microscopic dimensions. If this deformation occurs at elevated temperature and in the presence of air the intercrystalline surface thus exposed will become oxidized and

this film of oxide will prevent any subsequent rewelding or reunion of the surfaces so that the fractures become permanent. If this process of deformation is repeated these inter-crystalline fractures will finally result in the detachment of fine particles of oxidized lead.

It may be remarked that 27 indicates gas burners adapted to supply heat to the lead tape or ribbon.

It will be obvious to those skilled in the art 10 that modifications may be made in details of construction and procedure without departing from the spirit of the invention which is not limited to such matters or otherwise than the prior art and the appended claims may require. 15

I claim:

1. A method of making lead oxide powder from a long integral ribbon of metallic lead which consists in moving the ribbon endwise, progressively and repeatedly disturbing the structure at 20 the surface of the ribbon while at elevated temperature and in the presence of air and detaching fine particles of oxidized lead.

2. A method of making lead oxide powder which consists in deforming the structure at the 25 surface of an endwise traveling, long integral lead ribbon by mechanically working the ribbon in the presence of air and at high temperature.

3. A method of making lead oxide powder from a long integral ribbon of metallic lead which consists in traveling the ribbon endwise and forming a film of oxide on the surface of the ribbon and scaling the ribbon by progressively and repeatedly mechanically disturbing its surface 30 while at a high temperature and in the presence of air.

4. A method of making lead oxide powder from an endwise traveling ribbon of metallic lead which consists in microscopically cracking and oxidizing and scaling the surface of the lead ribbon by disturbing the surface of the lead ribbon at spaced intervals along its path while it is 35 at a high temperature and in the presence of air.

5. A method of making lead oxide powder

which consists in deforming the structure at the surface of a lead ribbon by alternately flexing and reflexing the ribbon in the presence of air and at elevated temperature.

6. A process for manufacturing lead oxide by continuously feeding a long, integral lead ribbon endwise, and disturbing the surface structure of the ribbon as by bending the ribbon back and forth in the presence of an oxidizing atmosphere.

7. A process for manufacturing lead oxide by continuously feeding a lead ribbon endwise and disturbing the surface structure of the ribbon by hammering the ribbon with a hammer in the presence of air and at an elevated temperature.

8. Apparatus for making a powdered oxide from an oxidizable material comprising, a stationary casing having inlet and outlet ports therein adapted to closely fit and restrict the escape of gas from around a long integral ribbon of said material passing through said ports, mechanical parts of said apparatus mounted in said casing and arranged to disturb the surface of said ribbon and to remove from the surface of said ribbon the powdered oxide so formed, and conduits for supplying an oxidizing atmosphere to said ribbon in said casing.

9. Apparatus for making a powdered oxide from an oxidizable material comprising, a stationary casing having inlet and outlet ports

30 therein arranged to closely fit and to restrict the escape of gas from around a long integral ribbon of said material passing through said ports and having an outlet port for the escape of powdered oxide from said casing by gravity, mechanical parts of said apparatus in said casing and arranged to convey and support said ribbon through said casing and to disturb the surface of said ribbon and to remove from the surface of said ribbon the powdered oxide so formed, and a conduit for introducing oxidizing atmosphere 35 into said casing and onto said ribbon in said casing.

JOSEPH LESTER WOODBRIDGE.